

# UNITED STATES PATENT OFFICE.

HERBERT ABRAHAM, OF NEW YORK, N. Y., ASSIGNOR TO THE RUBBEROID CO., A CORPORATION OF NEW JERSEY.

## SHOE-FILLER.

1,385,808.

Specification of Letters Patent.

Patented July 26, 1921.

No Drawing.

Application filed November 17, 1917. Serial No. 202,566.

To all whom it may concern:

Be it known that I, HERBERT ABRAHAM, a citizen of the United States, residing at the city, county, and State of New York, have 5 invented certain new and useful Improvements in Shoe-Fillers, of which the following is a specification.

My invention relates to an improved shoe 10 filler composed of bituminous material containing a relatively small percentage of non-felted fibers, the composition being of such a nature as to become plastic under the influence of heat.

A composition made according to my invention has great waterproofing properties 15 and resiliency and will prevent entrance of moisture through the sole of the shoe.

Heretofore shoe fillers composed of a 20 felted fabric saturated and coated with bituminous matter have been used. Such a filler must be stamped out by means of a die in the size required to completely fill the space within the welt of the shoe, and, accordingly, it is necessary to have a die corresponding 25 to each side and shape of shoe manufactured. These dies are very expensive and must be renewed from time to time as the style and shape of the shoes are changed. Furthermore, the felted fabric 30 must be supplied in different thicknesses to conform to the thickness of the insole.

My improved filler, consisting of bituminized non-felted fibers is adapted to be applied in a heated plastic condition. This 35 will enable the composition to be spread in place with a heated trowel or other suitable instrument so as to conform to the size and shape of the insole, thus dispensing with the use of dies or other shaping apparatus.

40 My composition consists broadly of bituminous matter mixed while in a heated state with ten to thirty per cent. by volume, of non-felted fibers. The fibers are preferably of short length and may be of mineral, animal 45 or vegetable origin, as, for example, asbestos fibers, disintegrated wood (known to the trade as wood pulp or wood flour), rag fibers, or animal fibers, such as wool, hair or the like. I have obtained very satisfactory 50 results by using an average of 20% by volume of such fibers. I state the percentages in terms of volume rather than of weight as the specific gravity of the fibers will vary, depending upon the type that is used.

It will be apparent to those skilled in the 55 art that the character and proportions of the ingredients of which my shoe filler is made may be varied without departing from the scope of my invention. For example, I have obtained satisfactory results with fillers made 60 according to the following formulas. It is to be understood, however, that I do not limit myself to those:

(A) Blown petroleum asphalt obtained 65 from semi-asphaltic petroleum having a fusing point of 180° Fahrenheit (ball and ring method), 66 $\frac{2}{3}$  per cent. by weight. Asbestos fibers varying between  $\frac{1}{16}$  and  $\frac{1}{4}$  inch in length (specific gravity 1.894) 33 $\frac{1}{3}$ % by weight, equivalent to 17.6% by volume. 70

(B) Gilsonite 20% by weight, residual oil 80% by weight. These are melted together, the resulting bituminous mixture having a fusing point of 150° Fahrenheit (ball and ring method). 78% by weight of this bituminous mixture is then mixed with 22% by weight of "wood flour" (specific gravity 0.975) which is equivalent to 22.6% by volume. 75

(C) Straight run steamed-distilled residuum asphalt from Mexican petroleum having a fusing point of 140° Fahrenheit (ball and ring method), mixed in a proportion of 85% by weight of the residuum with 15% by weight of disintegrated rag fibers (animal and vegetable fibers having a specific gravity of 0.852) equivalent to 17.6% by volume. 80

The finished composition may be either solid or semi-solid and of such a nature that 90 it will be readily amenable to the influence of heat, so that at a temperature range of from two hundred to four hundred degrees Fahrenheit, it will assume a plastic consistency which will enable it to be readily 95 trowled. These characteristics are regulated by the nature of bituminous material used, which should be so selected that when mixed with the fibers, the filler will not yield susceptibility to the pressure of the foot 100 in hot weather and ooze out of place, and on the other hand will be able to withstand low temperatures and the flexure of the sole without cracking or powdering. Instead of using a bituminous matrix, I may use a 105 product consisting of resinous matter brought to the proper consistency by means of fatty or oily substances either of animal

or vegetable origin. The resinous matrix may be used alone or in combination with bituminous matter.

What I claim is:

- 5 A waterproof shoe bottom filler, composed of bituminated non-felted fibers, which when heated within a range of from 200 to 400 de-

grees Fahrenheit will assume a plastic consistency, enabling it to be readily troweled into the cavity between the sole and insole 10 of a shoe, and which at atmospheric temperatures will regain a tough, resilient and pliable state.

HERBERT ABRAHAM.

It is hereby certified that the name of the assignee in Letters Patent No. 1,385,808, granted July 26, 1921, upon the application of Herbert Abraham, of New York, N. Y., for an improvement in "Shoe-Fillers," was erroneously written and printed as The Rubberoid Co., a Corporation of New Jersey, whereas said name should have been written and printed as *The Ruberoid Co., a Corporation of New Jersey*, as shown by the record of assignments in this office; and that the said Letters Patent should be read with this correction therein that the same may conform to the record of the case in the Patent Office.

Signed and sealed this 30th day of August, A. D., 1921.

[SEAL.]

KARL FENNING,

*Acting Commissioner of Patents.*

Cl. 106—3.